

## UNITED STATES PATENT OFFICE

2,231,160

INDUCTANCE CORE HAVING LOW NEGATIVE  
TEMPERATURE COEFFICIENT OF INDUCT-  
ANCE AND METHOD OF MAKING ITPaul Gottschalt, Berlin-Spandau, Germany, as-  
signor to Siemens & Halske Aktiengesellschaft,  
Siemensstadt, near Berlin, Germany, a corpo-  
ration of GermanyNo Drawing. Application April 18, 1938, Serial  
No. 204,926. In Germany April 17, 1937

4 Claims. (Cl. 175—21)

(Granted under the provisions of sec. 14, act of  
March 2, 1927; 357 O. G. 5)

The invention relates to a method for pro-  
ducing coil cores of magnetizable material.

For numerous purposes in the field of electrical  
communication, inductance coils are required, the  
inductance of which must not change more than  
to an extremely slight degree for long periods of  
time (T). In addition, it is often necessary to  
make exacting demands with respect to the tem-  
perature coefficient

relation (2) by arrangements at the coil, which  
offers more technical possibilities than is the case  
with the condenser.

The temperature coefficient of the condensers  
mostly in use in technical engineering is in gen-  
eral positive in accordance with the linear coef-  
ficient of expansion of the material employed, so  
that in most cases a negative temperature coef-  
ficient of the coil must be required. For instance,  
the frequently used mica condenser in ambient 5  
air may have the coefficient  $\alpha = +3 \times 10^{-5}$  10  
degree<sup>-1</sup>, so that for the coils to be connected  
with such condenser the coefficient  $\alpha = -3 \times 10^{-5}$   
degree<sup>-1</sup> is prescribed.

However, the usual coils employed in electrical 15  
communication, in particular the coils without  
ferromagnetic core, such as are common for very  
high frequencies (short waves), show in the great  
majority of cases a positive temperature coef-  
ficient  $\alpha_L$ . With such coils, therefore, special 20  
technical measures are necessary for obtaining a  
certain pre-given negative temperature coef-  
ficient, for instance,  $-3 \times 10^{-5}$  degree<sup>-1</sup>. A num-  
ber of such measures are known, yet they have  
considerable drawbacks, or are only suitable for 25  
a greatly limited special use of the coils.

The invention does away with these disadvan-  
tages. According to the invention the magnet  
core of inductance coils designed to meet the  
aforementioned requirements, is produced by 30  
mixing ferromagnetic powder and an insulating  
substance, and/or several ferromagnetic kinds of  
powder with differing temperature coefficients,  
and/or several thermoplastic binding materials,  
while maintaining a mutual proportion resulting 35  
in a total temperature coefficient of pre-given  
small value, and by squirting the thus prepared  
mixture to obtain the desired shape of the core.

According to a preferred embodiment of my in-  
vention, the ferromagnetic portion of the mixture 40  
to be squirted consists of carbonyl iron powder or  
contains carbonyl iron powder as the major com-  
ponent, i. e. in an amount of at least 50% as com-  
pared with the total weight of the ferromagnetic  
portion. Especially favorable results are obtained 45  
with 50 to 80% carbonyl iron powder and 50 to  
20% of an iron-nickel alloy of high magnetic per-  
meability. The latter alloy may consist of about  
78.5% nickel, the remainder iron. The insulating  
binder to be mixed with the ferromagnetic por- 50  
tion may consist of thermoplastic materials, pref-  
erably polystyrol and the like. The binder is to  
be used in a proportion of 1/10 to 5/10 as com-  
pared with the weight of the ferromagnetic por- 55  
tion. If normal polystyrol is employed, propor-

$$10 \quad \alpha = \frac{1}{L} \frac{\partial L}{\partial T}$$

of the inductance (L). There are cases where as  
small a temperature coefficient as possible is de-  
sired, for instance,  $\alpha < 1 \times 10^{-5}$  degree<sup>-1</sup>; but more  
often it is required that the temperature coef-  
ficient come as near as possible to a certain pre-  
given value, for instance,  $\alpha = -3 \times 10^{-5}$  degree<sup>-1</sup>.  
Such a given value, usually negative, of the tem-  
perature coefficient is required especially in such  
cases where the coils are to be arranged in oscil-  
lating circuits, band filters and similar connec-  
tions with condenser circuits, and where the nat-  
ural frequencies of these coil-condenser-circuits  
are supposed to have a high constancy and a  
slight dependence on temperature. These nat-  
ural frequencies  $f_0$  depend, in general, on the in-  
ductance (L) of the coil and the capacity (C) of  
the condenser in accordance with the relation

$$30 \quad f_0 = \frac{1}{2\pi\sqrt{LC}} \quad (1)$$

The often necessary high constancy of the nat-  
ural frequency  $f_0$  is obviously attained if—

35 (1) L and C at any maintained temperature T  
remain unchanged in time within the tempera-  
ture range met with in regular service, and if

(2) Within this entire range of temperature  
the temperature coefficient

$$40 \quad \alpha_L = \frac{1}{L} \frac{\partial L}{\partial T}$$

of the coils with reversed signs corresponds to  
that of the temperature coefficient

$$45 \quad \alpha_C = \frac{1}{C} \frac{\partial C}{\partial T}$$

of the condenser, viz., if the relation

$$50 \quad \alpha_L = -\alpha_C \quad (2)$$

is complied with.

Since the temperature coefficient of a condenser  
can, in general, be intentionally influenced only  
by comparatively troublesome and expensive  
measures, it is usually endeavoured to satisfy the

tions between 2/10 and 5/10 have proved favorable, while when polystyrol of higher molecular weight is used, a proportion between 1/10 and 3/10 is preferable.

- 5 For elucidating the invention, some comparative examples of differently produced mass cores commonly used for Pupin coils, and the dependence of the inductance on the temperature for a number of temperature changes are referred to in 10 the following. As Example No. 1, a core made of carbonyl iron powder and insulated by organic substances is taken in view; and as Example No. 2 a core made of ferro-nickel alloy powder, which has been insulated with glow-resistant inorganic 15 substances, and after the pressing has been annealed in known manner at about 500°.

A mass core according to Example No. 1, is unsuited for coils of high constancy from the outset, owing to its considerable want of reproductive 20 capacity, i. e. the material and permanent alterations after repeated changes of temperature. The temperature coefficient, while negative, is too large ( $\alpha_L = -17 \times 10^{-5}$  degree  $^{-1}$ ). In the case of Example No. 2, the want of reproductive 25 capacity is considerably less, but the temperature coefficient is highly positive

$$(\alpha_L = +23 \times 10^{-5} \text{ degree } ^{-1})$$

It has further been found, that the constancy in 30 time of all those cores, which have been produced by mechanical pressing together of the insulated powder, cannot be increased at all, or only under considerable difficulties, to the extent frequently required.

35 While it is known to produce mass cores not by purely mechanical pressing-together, but by die casting, such mass cores do not offhand yield the low magnitudes of the temperature coefficient required in each case. It has however been 40 found—and this recognition forms a basis of the present invention—that with cores produced by the die casting method in fact a better constancy in time can be attained, than with the cores produced up to now principally by the 45 pressing method.

As Example No. 3, a magnet coil may be considered, having a core squirted in known manner of carbonyl iron. Such a coil shows fewer 50 changes in its inductance with repeated changes of temperature, i. e. the want of reproductive capacity is greatly reduced as compared with that according to Example No. 1. The temperature coefficient is, in fact, negative, as generally required, but not to the desired amount of about

$$\alpha_L = -3 \times 10^{-5} \text{ degree } ^{-1}$$

55 As compared with the foregoing three types of cores, a material advance with respect to constancy in time and reproductive capacity, together with a low magnitude of the temperature coefficient, is obtained if the cores are produced according to the invention by employing certain mixture proportions and producing the cores by squirting. An inductance coil having such a core, shows, for instance, a temperature coefficient of the desired value  $\alpha = -3 \times 10^{-5}$  degree  $^{-1}$ , and suffers practically no changes of this value during a period of several months, i. e. such changes remain materially below  $\pm 1 \times 10^{-4}$ .

A method of producing such cores is the following. 60% carbonyl iron powder is mixed with 40% powder of a ferro-nickel alloy containing 78.5% nickel contents. This powder mixture is pre-insulated in the usual manner with a thin layer of insulating material, then mixed with 15 75 weight units of polystyrol powder and eventually

formed in known manner into annular cores by squirting. By altering the mixture proportions, i. e. of the iron and alloy mixture or of the metal and polystyrol mixture or of both proportions, the temperature coefficient can be changed at will 5 within limits wide enough to allow satisfying all conditions actually occurring in practice. In each particular case, the most favorable mixture proportions may be computed by an interpolation based upon the measured temperature coefficients 10 of known cores with similar mixture proportions, or may be newly determined by measurings of cores with differing mixture proportions.

In order to obtain as high permeabilities as possible, it is preferable to choose as high a share 15 of ferromagnetic powder as possible, as long as this does not noticeably impair the capability of being squirted, and to vary the magnitude of the temperature coefficient by correspondingly varying the mixture proportion between two differing 20 kinds of ferromagnetic powder.

But there exist also fields of application, in particular with regard to coils for very high working frequencies, for instance short waves, where very slight permeabilities are desired owing 25 to the unavoidable losses in the iron core increasing with the frequency. In cases of this nature the required temperature coefficient can be obtained by using a greater share of insulating material, or also, without the use of different 30 kinds of ferromagnetic powder, merely by exactly maintaining a mixture proportion between a ferromagnetic powder and a thermoplastic mass, which proportion may be determined in a given case, for instance, by some tests made with cores 35 of different mixture proportions.

Surprisingly favorable results are obtained not only by the heretofore customary polystyrol, but by similar thermoplastic masses, which, however, have a higher thermal stability. Squirted mass 40 cores of carbonyl iron powder and a polystyrol, having an extremely high mean molecular weight of, for instance, more than 100,000, resulted in very slight temperature coefficients and a good 45 constancy in time. Coils with annular cores made 45 of a mixture with 15 weight units of this polystyrol to 100 units of iron showed by measurements the small value  $\alpha_L = -4 \times 10^{-5}$  degree  $^{-1}$ , and coils with other core shapes of the same core substance showed values between  $\alpha_L = -2 \times 10^{-5}$  50 degree  $^{-1}$  and  $\alpha_L = -5 \times 10^{-5}$  degree  $^{-1}$ .

Further, the temperature coefficient may also be affected in the manner desired by the simultaneous use of different thermoplastic masses in certain mixture proportions, for instance, by mixing 55 a part of the said polystyrol, having a high molecular weight, with normal polystyrol. The use of polyvinyl-carbazal has also yielded very good results.

Physical examinations conducted in order to 60 find an explanation of the causes for the improvement obtained by the invention, have shown that the better constancy in time and the improved reproductive capacity of the cores is due to the thorough bond of the iron powder with the insulating substance effected by the squirting method and that the effect of the mixture proportion on the temperature coefficient is due in particular to the thermic coefficient of expansion.

What is claimed is:

1. The method of producing magnetizable cores for inductance coils having a temperature coefficient of inductance of pre-given negative value and high constancy in time, comprising the steps of mixing a powdered ferromagnetic material 75

consisting of at least 50% of carbonyl iron powder with an insulating binder composed of polystyrol powder of normal molecular weight and polystyrol powder of a higher mean molecular weight, said powders being employed in a mutual proportion of weight designed for resulting in a temperature coefficient of pre-given negative value, and shaping said mixture by squiring.

2. A magnet core consisting of a squirted mixture of a ferromagnetic mass composed of 50 to 80% carbonyl iron powder and 50 to 20% powder of an iron-nickel alloy with about 78.5% nickel with an insulating binder containing polystyrol substances of different molecular weight, and characterized by a low negative temperature coefficient of inductance and high constancy in time of said coefficient.

3. A magnet core consisting of a squirted mixture consisting of a ferromagnetic mass composed

of carbonyl iron powder and a powdered iron-nickel alloy of high magnetic permeability, and of an insulating thermoplastic binder consisting substantially of polystyrol, said binder forming  $\frac{1}{6}$  to  $\frac{1}{8}$  in weight as compared with the weight of said ferromagnetic mass, and characterized by a low negative temperature coefficient of inductance and high constancy in time of said coefficient.

4. A magnet core consisting of a squirted mixture of ferromagnetic mass and an insulating binder, said ferromagnetic mass being composed of 50 to 80% carbonyl iron powder and 50 to 20% powder of an iron-nickel alloy with about 78.5% nickel, and said binder consisting of polystyrol and weighing  $\frac{1}{6}$  to  $\frac{1}{2}$  of the weight of said ferromagnetic mass.

PAUL GOTTSCHALT.